

Oct. 23, 1951

W. R. PATTERSON

2,572,754

INGOT MOLD SPLASH BOWL

Filed Feb. 28, 1949

FIG. 1.



FIG. 5.



FIG. 4.



FIG. 3.



FIG. 2.



WILLIAM R. PATTERSON

*Lyons & Lyons*  
ATTORNEYS

## UNITED STATES PATENT OFFICE

2,572,754

## INGOT MOLD SPLASH BOWL

William R. Patterson, Los Angeles, Calif., assignor  
to The National Supply Company, Pittsburgh,  
Pa., a corporation of Pennsylvania

Application February 28, 1949, Serial No. 78,777

6 Claims. (Cl. 22—148)

1

This invention relates to the manufacture of metal ingots.

Big end up ingots which are poured from the top are commonly subject to surface defects caused by splashing of the stream of molten metal from the bottom of the mold at the beginning of the pouring operation. The splashing metal which strikes the relatively cold side walls of the mold results in formation of solidified plate-like masses which may adhere to the mold. The stream of hot metal from the nozzle of the pouring ladle falls a considerable distance, particularly in the case of tall ingot molds. The molten metal strikes the bottom of the mold with considerable force and a very strong splash may result if the molten metal stream impinges on a surface normal to the direction of the stream. As the pouring continues and as the level of the molten metal rises in the mold, the frozen plate-like masses are covered by molten metal and may partially fuse into the liquid mass. These partially fused masses are poorly bonded and become what is commonly known as "scabs." These give appreciable trouble in the production of forged or rolled products made from such an imperfect ingot. Furthermore, these chilled masses of metal may not adhere to the mold walls but may detach themselves and locate in the body of the ingot and thus adversely affect the quality of the ingot.

Surface scabs and internal defects of this character are found in top poured ingots made in either closed bottom molds or open bottom molds, but the most serious trouble is encountered with the open bottom molds since the shape of the bottom is generally made substantially flat. It is customary to place the bottom of the open bottom mold on a substantially flat plate known in the art as a stool plate. This surface is normal to the molten stream of metal as it enters the mold, and hence highly undesirable vigorous splashing occurs.

It is the principal object of my invention to minimize the splashing of molten metal as it is initially poured into the upper end of either closed bottom or open bottom molds.

Another object is to provide a splash bowl for an ingot mold provided with means for absorbing the kinetic energy of the stream of molten metal to minimize splashing.

A more particular object is to provide a splash trap of this type with a plurality of upwardly extending spikes arranged to dissipate the energy of the stream of molten metal and to form a pool to cushion the falling stream.

2

Other detailed objects and advantages will appear hereinafter.

In the drawings:

Figure 1 is a sectional elevation showing a preferred embodiment of my invention as applied to an open bottom ingot mold of the type producing big end up ingots.

Figure 2 is a sectional plan view taken substantially on the lines 2—2 as shown in Figure 1.

Figure 3 is a top plan view of a splash bowl employed in connection with my invention.

Figure 4 is a sectional elevation taken substantially on the lines 4—4 as shown in Figure 3.

Figure 5 is a side elevation partly in vertical section illustrating an embodiment of my invention in connection with a closed bottom ingot mold.

Referring to the drawings, the ingot mold 10 is of the open bottom type and the molten stream 20 of metal is poured into the upper end from any suitable ladle (not shown). The central opening 11 in the mold 10 may be noncircular as shown clearly in Figure 2 in order to produce a fluted ingot. This central opening is tapered for a major portion of the height of the mold 10 so that the cross-sectional size of the opening is smaller near the bottom of the mold 10.

The mold 10 is adapted to rest on a stool plate 12 having a central opening 13. The upper end 30 of this opening 13 may be flared to receive the conical periphery 14 of the splash bowl 15. The opening in the lower end of the ingot mold 10 is constricted as shown at 16 so that the extreme lower end of the opening is substantially 35 in alignment with the upper end of the opening 13 in the stool plate 12. The splash bowl 15 is provided with a central cavity 17 forming a continuation of the opening 11 in the ingot mold 10. A plurality of vertical spikes 18 formed integrally with the bottom 22 of the splash bowl 15 extend upwardly into the cavity 17. When the molten stream of metal is poured into the opening 11 the stream falls vertically into the cavity 17. The vigorous splashing which would normally 40 occur on a flat horizontal surface does not take place and the energy of the stream is dissipated as it bounds and rebounds among the vertical spikes 18. A pool of molten metal is thus formed in the cavity 17 and in the lower end of the central opening 11 without any objectionable 45 splashing of molten metal upwardly onto the sides 19 of the opening 11 in the ingot mold 10. Once this cushioning pool has been formed the function of the spikes 18 has been accomplished, 50 and thereafter the molten pool prevents any

serious splashing upwardly onto the relatively cold walls of the mold.

The spikes 18 may fuse into the molten metal as it solidifies and the splash bowl 15 may become attached to the small end of the solidified ingot. This does not, however, present any problem because the small end of the ingot is cropped off in the region of the restricted throat 16. While a new splash bowl is normally required for each ingot poured into the mold, this relatively small additional cost is more than offset by the savings in surface chipping and conditioning of the ingot prior to rolling or forging. Furthermore, the internal quality of the ingot metal is superior because of the freedom from partially fused splash metal which may have adhered initially to the mold walls but later become detached and located within the body of the ingot.

The ingot mold 10 and splash plate 12 may be provided with the usual lugs 20 for handling.

The embodiment of my invention shown in Figure 5 utilizes a splash bowl 30 which is substantially the same as that described in the previous embodiment. The splash bowl 30 is mounted directly in the tapered opening 31 formed in the bottom of the closed bottom ingot mold 32. In this embodiment no stool plate is employed. The action of the spikes 33 on the splash bowl 30 is substantially the same as that described above. In either case the energy of the molten metal stream is diffused and a minimum of splashing occurs whether the stream falls directly into the center of the splash bowl or somewhat off-center.

While it is not essential that the spikes be parallel in order to accomplish the benefits of my invention, nevertheless, I prefer to form them in parallel relationship for ease of manufacture. The spikes 18 may be conveniently cast integrally with the walls and bottom of the bowl 15.

Having fully described my invention, it is to be understood that I do not wish to be limited to the details herein set forth, but my invention is of the full scope of the appended claims.

I claim:

1. Apparatus for casting metal ingots comprising an upright mold having a central opening to receive a stream of molten metal, and a splash minimizing bowl member forming the lower end of the mold having a plurality of integral upwardly extending spikes adapted to diffuse the energy of the molten stream falling thereon to minimize splashing of metal upwardly against the sides of the mold opening.

2. A combined splash bowl and bottom plug for an ingot mold, the bowl having walls and an integral floor defining an upwardly opening cavity, the walls and floor being sufficiently massive to withstand pressure of liquid metal in the mold, and a cluster of spikes formed integrally with the floor and extending upwardly into the said cavity.

3. Apparatus for casting metal ingots comprising in combination an upright mold having a

central opening extending therethrough to receive a stream of molten metal, a splash bowl insertable through the mold opening to form a plug at the bottom thereof, the splash bowl having walls and a floor formed integrally therewith to define an upwardly opening cavity, and a plurality of spikes fixed on the floor and extending upwardly into the cavity.

4. Apparatus for casting metal ingots comprising an upright mold having a central opening extending therethrough to receive a stream of molten metal, a stool plate supporting the mold and provided with a central aperture, a massive splash bowl resting on the stool plate in said aperture and forming the lower end of the mold opening, the splash bowl having walls and a floor formed integrally therewith to define an upwardly opening cavity, and a plurality of spikes fixed on the floor and extending upwardly into the cavity.

5. Apparatus for casting metal ingots comprising an upright mold having a central opening extending therethrough to receive a stream of molten metal, a stool plate supporting the mold and provided with a central tapered aperture, a massive splash bowl having externally tapered walls received in said aperture, the bowl also having a floor integrally joining the walls, and a plurality of spikes extending upwardly from the floor of the bowl.

6. In an apparatus for casting metal ingots, including an upright mold having a central opening extending therethrough to receive a stream of molten metal, and a stool plate supporting the mold and provided with a central aperture having tapered walls, the improvement comprising: a massive splash bowl having a tapered external surface adapted to fit within said tapered walls, the splash bowl forming the lower end of the mold opening, the splash bowl having walls and a floor formed integrally therewith to define an outwardly opening cavity, and a plurality of spikes fixed on the floor and extending upwardly into the cavity.

45 WILLIAM R. PATTERSON.

#### REFERENCES CITED

The following references are of record in the file of this patent:

#### 50 UNITED STATES PATENTS

| Number       | Name     | Date           |
|--------------|----------|----------------|
| 728,552      | Dixon    | May 19, 1903   |
| 1,570,473    | Gathmann | Jan. 19, 1926  |
| 55 2,054,597 | Gathmann | Sept. 15, 1936 |
| 2,444,140    | Messler  | June 29, 1948  |
| 2,453,643    | Schmertz | Nov. 9, 1948   |

#### FOREIGN PATENTS

| Number  | Country       | Date          |
|---------|---------------|---------------|
| 415,031 | Great Britain | Aug. 13, 1934 |
| 316,164 | Germany       | Nov. 22, 1919 |